

## 1

3,071,462

## MAGNESIUM ALLOYS

Geoffrey Charles Edward Olds, Leicester, England, assignor to Associated Electrical Industries (Rugby) Limited (formerly known as The British Thomson-Houston Company Limited), London, England, a British company

No Drawing. Filed July 15, 1960, Ser. No. 42,985  
3 Claims. (Cl. 75—168)

The present application is a continuation-in-part of application Serial No. 768,062, filed on October 20, 1958, by me and assigned to the assignee of the present application.

This invention relates to magnesium alloys suitable, inter alia, for use as a canning material for the fuel elements of nuclear reactors. For such purpose, the alloy initially cast is required to be subjected to mechanical working whereby it is wrought into a form suitable for the required application. This may be effected by hot extrusion.

The important mechanical properties required in an alloy to be used as a canning material for uranium fuel in a thermal nuclear reactor are high creep ductility between 200° C. and 500° C.; small grain size and high stability of grain size up to 500° C.; freedom from excessive intercrystalline cavitation; high creep strength at low stresses at the highest operating temperatures and good weldability.

Alloys used for cans in natural uranium reactors must also possess very low neutron absorption cross-sections and for this reason magnesium is the most important metal to form the main constituent of any alloy used. Any alloying elements used must be such that the neutron absorption cross-section of the resulting alloy is adequately small. Magnesium alloys which have been considered up to now have been those in which the main alloying constituent is approximately 1% aluminum, magnesium alloys containing 0.5% zirconium, and those containing 0.5% zirconium and 0.5—1% zinc.

The two alloys of magnesium with 0.5% zirconium, and magnesium with 0.5% zirconium and 0.5—1% zinc have many properties which make them suitable for reactor cans with the exception that their creep strength at high temperatures of the order 500° C. is insufficiently high.

I have found that a small quantity of manganese alloyed in magnesium with zirconium produces an alloy with high creep resistance, yet still possessing the other desirable properties which are known to exist in binary magnesium-zirconium or ternary magnesium-zirconium-zinc alloys. These improved alloys are basically single-phase alloys, which at high temperatures do not exhibit precipitation hardening which is usually associated with creep resistance.

An alloy according to the invention consists of zirconium, magnesium and manganese, the proportions, by weight, in the alloy being 0.5—1.0% Zr, 0.05—0.5% Mn, and the remainder magnesium.

It is known that the useful liquid and solid solubility of Zr in Mg to form a single phase alloy is about 1.0%, above which percentage a zirconium precipitate is present in the final alloy. Also manganese has a limited liquid and solid solubility in magnesium, such that if the amount present in a binary alloy exceeds about 0.5% an undesirable precipitate is present in the alloy, which may lead to embrittlement. If Zr and Mn are both present in an Mg alloy, each of the two elements limits the solubility of the other, i.e. a small Mn addition of a few tenths of 1% reduces the solubility of Zr to less than 1.0%. The incorporation of Mn in the manufacture of Mg-Zr alloys therefore necessitates the reduction of the Zr con-

## 2

tent to less than 1.0%, both on grounds of obtaining the alloy elements in solution in the melt, and in producing a final alloy of single phase, which for the latter reason should also be free from serious embrittlement. The Zr and Mn contents of any Mg-Zr-Mn alloys are, therefore, interdependent.

Furthermore, the preferred maximum Mn content for a canning material on grounds of neutron absorption economy is about 0.2%.

10 In more detail, the following examples are given of preferred compositions which were found to be basically single phase alloys.

Alloy (1): 0.6% Zr, 0.1% Mn, remainder Mg.

15 Alloy (2): 0.7% Zr, 0.27% Mn, remainder Mg.

The improvement in creep resistance of alloy (1) containing manganese over its parent alloy of Mg-Zr and over alloy (A) of lower content of zirconium is shown by tensile test creep results as follows:

20

| 25                | Alloy | Composition |      | Secondary creep rate at 1,000 hours' duration at 450° C. at stress of 100 p.s.i., strain/hour |
|-------------------|-------|-------------|------|-----------------------------------------------------------------------------------------------|
|                   |       | Zr          | Mn   |                                                                                               |
| Parent Mg.Zr..... |       | 0.6         |      | 68×10 <sup>-6</sup>                                                                           |
| Alloy A.....      |       | 0.5         | 0.11 | 0.6×10 <sup>-6</sup>                                                                          |
| Alloy 1.....      |       | 0.6         | 0.1  | 0.2×10 <sup>-6</sup>                                                                          |

Creep tests under more severe conditions at 50 p.s.i. and 500° C. show that alloy (2) is superior to alloy (1) and also to alloy (B) of similar Mn and lower Zr content, even when the latter alloy was tested at a lower stress.

| 40             | Alloy | Composition, percent |      | Stress, p.s.i. | Secondary creep rate at 1,000 hours' duration at 500° C., strain/hour |
|----------------|-------|----------------------|------|----------------|-----------------------------------------------------------------------|
|                |       | Zr                   | Mn   |                |                                                                       |
| Alloy (B)..... |       | 0.37                 | 0.24 | 15             | 1.5×10 <sup>-6</sup>                                                  |
| Alloy (1)..... |       | 0.6                  | 0.1  | 50             | 18×10 <sup>-6</sup>                                                   |
| Alloy (2)..... |       | 0.7                  | 0.27 | 50             | 0.4×10 <sup>-6</sup>                                                  |

The above data demonstrate that Mg-Zr-Mn alloys containing 0.6% and 0.7% Zr are superior to the parent Mg-0.6% Zr alloy. At Mn levels of approximately 0.1% and approximately 0.25%, the data also show that contents of Zr of 0.6% and 0.7% respectively give higher creep strengths than similar alloys containing less than or equal to 0.5% Zr.

55 The following test data show that alloys (1) and (2) possess a small grain size, free from excessive growth at 500° C., and exhibit adequate tensile ductility at 200° C.:

| 60                | Alloy | Initial average grain diameter in microns | Average grain diameter in microns after annealing 500 hours at 500° C. | Percent tensile elongation at fracture when strained at 1% per hr. at 200° C.   |                                                                                 |
|-------------------|-------|-------------------------------------------|------------------------------------------------------------------------|---------------------------------------------------------------------------------|---------------------------------------------------------------------------------|
|                   |       |                                           |                                                                        | Percent tensile elongation at fracture when strained at 0.1% per hr. at 200° C. | Percent tensile elongation at fracture when strained at 0.1% per hr. at 200° C. |
| Parent Mg.Zr..... |       | 32                                        | 97                                                                     | 77                                                                              | 76                                                                              |
| Alloy (1).....    |       | 25                                        | 35                                                                     | 49                                                                              | 41                                                                              |
| Alloy (2).....    |       | 37                                        | 60                                                                     | 85                                                                              | 41                                                                              |

What I claim is:

1. An alloy consisting of magnesium, zirconium and

manganese, the proportions, by weight, of the constituents of the alloy being 0.6 to 0.7% zirconium, 0.1 to 0.27% manganese, and the remainder wholly magnesium except for unavoidable impurities.

2. An alloy consisting essentially, by weight, of zirconium 0.6%, manganese 0.1%, and the remainder magnesium except for unavoidable impurities.

3. An alloy consisting essentially, by weight, of zirconium 0.7%, manganese 0.27%, and the remainder magnesium except for unavoidable impurities.

5

10

## References Cited in the file of this patent

## FOREIGN PATENTS

806,104 Great Britain ----- Dec. 17, 1958

## OTHER REFERENCES

"Influence of Zirconium upon the Solidification of Magnesium Alloys and Some of the Properties of Magnesium Alloys Containing Zirconium," by Franz Sauerwald, Zeitschrift für Metallkunde, vol. 40, 1949, pp. 44 and 45.